

Feb. 25, 1941.

S. MUSHER

2,233,142

PAPER PACKAGING MATERIAL AND METHOD OF MAKING THE SAME

Filed May 29, 1939

Fig. 1.



Fig. 2.



Fig. 3.



INVENTOR

Sidney Musher

BY

*Harry Price*  
ATTORNEY

## UNITED STATES PATENT OFFICE

2,233,142

PAPER PACKAGING MATERIAL AND  
METHOD OF MAKING THE SAMESidney Musher, New York, N. Y., assignor to  
Musher Foundation Incorporated, New York,  
N. Y., a corporation of New York

Application May 29, 1939, Serial No. 276,413

9 Claims. (Cl. 91—68)

This invention relates to an improved paper sheet wrapping material capable of prolonging the life of packaged organic compositions and particularly when such compositions contain 5 glyceride oils and fats.

Flexible paper packaging materials such as parchment, greaseproof, glassine, sulfite, etc., papers and boards, whether made by the sulfite or sulfate processes have substantially no protective properties with respect to organic packaged compositions. Such papers and boards are, however, used for the packaging of materials of the nature of lard or other shortening, crackers, 10 cookies, cakes and cookery products, milk, orange juice, butter, candies and confections, ice cream, cheese, bacon, hams, beef, oranges, lemons and other citrus fruit, corn flakes, wheat cakes, shredded wheat, nuts, potato chips, etc., all of 15 which are subject to oxidative deterioration and development of objectionable off-odors and flavors during normal storage or distribution.

In addition, the entrained air in the package readily accelerates this deterioration for it is not practicable, where cellulosic packaging materials 20 are used, for the packaged product to be held under vacuum or under inert gases such as nitrogen, carbon dioxide, etc.

An object of this invention is, therefore, the 25 production of improved paper packaging materials which will prolong the life of packaged organic compositions and which will be readily acceptable for use in conjunction with food compositions and without objection by health and governmental agencies.

Still further objects and advantages will appear from the more detailed description set forth below, it being understood, however, that this more detailed description is given by way of illustration and explanation only, and not by way 30 of limitation, since various changes therein may be made by those skilled in the art without departing from the scope and spirit of the present invention.

In accordance with this invention, it has surprisingly been found that certain materials applied to paper wrappers will substantially balance 35 the effect of the air and the naturally oxidizable characteristics of the packaged organic composition.

It has, furthermore, been surprisingly found 40 that this protection can be secured if only the edges of the packaged composition are in contact with the treated paper material, the major portion of the surface of said packaged composition being in contact with air. For example, less than

10% of the total surface area of the packaged composition may be in contact with the sheet packaging material and 90% or more in contact with air, but stabilization against oxidative deterioration is nevertheless obtained. 5

In accomplishing the results of this invention, there are preferably applied certain di-substituted benzenes to the paper packaging material, the substances most satisfactorily employed being the hydroxy di-substituted benzenes, preferably in para position, and less preferably the hydroxy di-substituted naphthalenes. As a general rule, these substances should contain not more than 14 carbon atoms and preferably not over 10 carbon atoms. 10

Apparently these compounds form some combination with the cellulose of the paper packaging materials, such combination being of a physical or chemical nature, with the result that the combination of the paper material and the aromatic compound has been activated to develop 15 marked antioxygenic and stabilizing activity.

In applying these aromatic compounds to the packaging material, it has been found most suitable to apply them with non-oxidizing substantially neutral sizing materials, and particularly with hydroxylated aliphatic compounds as these aid most satisfactorily in obtaining the desired results, such sizing materials including glycerine 20 and its related sizing compounds, carbohydrates such as starch and sugars, dextrin and carbohydrate gums such as gum arabic, karaya, tragacanth, etc. 25

Less preferably there may be utilized as the sizing carrier the high molecular weight proteins 30 and protein containing materials such as casein, soya proteins, partly or wholly coagulated gelatin or glue, etc.

The stabilizing aromatic compounds are preferably applied in amounts ranging from 0.001% 35 to 1% against the weight of the paper sheet packaging material. Generally, about 0.05% to 0.25% by weight is the desired amount to give satisfactory protection. 40

The preferred aromatic hydroxy compound to use in accordance with this invention is hydroquinone. Other useful di and tri-hydroxy compounds, the hydroxy groups of which may have been etherized, include guaiacol, phloroglucinol, resorcinol, pyrogallol, tyrosine, eugenol, thymol, 45 vanillin, gallic acid and gallotannin.

The hydroquinone should be applied to the paper so that it is present at the surface of that paper and desirably spread out in a thin film at the surface of the paper and on that surface 50

which is to be placed into contact with the edges of the packaged product.

As an example of the method by which the hydroquinone or similar compound may be applied, it may be added to the tub sizing tanks through which the paper or paperboard passes, using from 0.5% to 15% of the hydroquinone against the weight of the water and other materials contained in the size. About 2% of hydroquinone against the weight of the size is a satisfactory amount. When the sheet material, whether it be parchment paper, sulfite paper, greaseproof paper, glassine paper, prime stock or secondary stock board, passes through the sizing tank containing the hydroquinone, sufficient of the hydroquinone will be picked up on the sheet to give marked stabilizing activity to packaged organic compositions.

A particularly desirable method for the application of the hydroquinone to the sheet is first to admix it with a carrier as indicated above. For example, to tapioca or corn starch may be added from 0.5% to 5% by weight of hydroquinone and thoroughly admixed therein. Where desired, the starch may then be boiled or treated with an enzyme to prepare for sizing and utilized in the sizing troughs for application to the packaging material.

Desirably, the paper or board may be allowed to pass through the sizing trough so that a portion of the hydroquinone adheres to the surface of the paper or board. In the case of parchment paper, the hydroquinone may desirably be present in the sizing troughs through which the paper passes after the sulfuric acid and alkali neutralization parchmentizing operation.

By utilizing a starch as a carrier for the hydroquinone, the individual particles of the hydroquinone are sufficiently well dispersed throughout the tub carrying the size so that the paper or board which passes through it picks up a uniform quantity of the hydroquinone.

#### EXAMPLE I

45 A 30 lb. stock greaseproof paper was passed through a bath consisting of 95% water and 5% hydroquinone. The paper was then dried in a vacuum oven at 65° C., it being estimated that 0.1% of hydroquinone against the weight of the paper was applied. The paper thus made was used for the packaging of soda crackers, only the edges of which were in contact with the paper and about 98% of the surface of the crackers being exposed to air. The crackers thus packaged were compared in keeping quality with crackers packaged in ordinary untreated greaseproof paper by holding in the dark at 98° F. and observing for rancidity.

60 Rancidity observed after  
Crackers in untreated paper----- 9 days  
Crackers in treated paper----- 16 days

#### EXAMPLE II

65 A preboiled dried powdered corn starch was thoroughly mixed with 5% by weight of hydroquinone. The starch containing the hydroquinone was sized on glassine paper by passing the paper before supercalendering through a size bath containing 92% water and 8% of the starch-hydroquinone combination. The paper was then supercalendered and dried. This treated glassine was made into bags and used for the packaging of potato chips, only a portion of the edges of a minor number of which were in 75 actual contact with the paper. The potato chips

thus packaged and held in the dark at 98° F. were free of objectionable rancidity for over twice as long as a similar lot of potato chips packaged in ordinary untreated glassine and held under similar conditions of storage. 5

This method of treating paper to retard oxidative deterioration of packaged products is in no way related to the filtering out of any special light rays since the desired results are obtained even where no transmission of light is involved 10 and the packaged composition is stored in the dark away from all light rays. Moreover, the protective materials of the instant invention are incapable of producing any special light filtration benefits. 15

The process of the present invention is particularly concerned with the treatment of those papers and boards which are normally opaque and are not changed in color by this treatment.

The process of the present invention is most 20 particularly of value in connection with the plain (non-regenerated) types of papers and boards whereby no hard surface film is present. Where a hard surface film of the nature of the regenerated cellulosic films, resinous sizing materials, 25 etc., is utilized, the results of the present invention are not readily obtained and most desirably, the treatment of the present invention should be given to ordinary absorbent paper and board.

Surprisingly, it has been found that the treat- 30 ment of paper with hydroquinone in the manner indicated will show even better results than where the same amount of hydroquinone is added to the packaged composition.

#### EXAMPLE III

##### Crackers A

To 1000 grams of cracker dough containing 120 grams of bleached lard was added 0.01 gram of hydroquinone. The crackers were baked, 40 packaged 3 crackers to each package with ordinary parchment paper and stored in the dark at 98° F. until rancidity was detected.

##### Crackers B

45 1000 grams of the same cracker dough but without the hydroquinone were used in the manufacture of crackers, the crackers baked and packaged, using 3 crackers to each package, 50 with parchment paper. In this case one side of the parchment paper had previously been soaked with water containing 0.01 gram of hydroquinone until all the water plus the hydroquinone was adsorbed on the paper, and the paper was then dried with the hydroquinone present 55 on the surface of that side of the paper which would be adjacent to the edges of the crackers when wrapped. These crackers were tested in the same manner as Crackers A. 60

In both cases only about 2% of the total surface area of the crackers was exposed to the parchment paper, the balance being exposed to air.

Observations for rancidity were made with 65 the following results:

|                 |                      |
|-----------------|----------------------|
| Crackers A----- | Rancid after 31 days |
| Crackers B----- | 45 days              |

#### EXAMPLE IV

A mixture was prepared comprising 1% of hydroquinone and 99% of tapioca starch by weight. The starch-hydroquinone combination was gelatinized by boiling in 7 times its weight 75

of water and then sufficient additional water was added so that only 6% of the gelatinized starch-hydroquinone combination was present in the water. Board made of sulphite secondary stock was passed through this bath and the board was then heated to 220° F. until thoroughly dry. The board thus made was used for the packaging of sweet wafers, only the edges of which touched the board. The wafers thus packaged were found to be extremely resistant to rancidity and to the development of carton odors and tastes.

The protection afforded is of particular value in view of the fact that the addition of hydroquinone to crackers would be prohibited because of the questionable edibility of that product whereas, in accordance with this invention, the hydroquinone may be utilized without question by food authorities.

Furthermore, it is not well understood as to why the presence of hydroquinone on the paper should be so much more effective than where it is added to and dispersed in the packaged composition.

The present specification and claims are limited to those papers that are sized or coated with wax, paraffin, hydrogenated fat or similar surface coatings of non-resinous character. The hydroquinone is applied to the paper or board and the paper or board then waxed or paraffined, and such paper or board will retain its protective properties in the same way and even in a more effective way than if the hydroquinone had been mixed with the paraffin or dusted over the surface of the paraffin.

Surprisingly, the paraffin or wax covering over the hydroquinone whereby the hydroquinone is kept from contact with the packaged composition presents no barrier to giving substantial protection to packaged oil or fat containing organic compositions. Such papers or boards are, after the application of the hydroquinone as a sizing, surface coated with paraffin or impregnated with paraffin oils and utilized in the packaging of milk, 45 orange juice, meats, fish and poultry for storage, biscuits and crackers, caramels and candies, etc.

#### EXAMPLE V

A sulfite paper was sized with hydroquinone in the manner described in Example I. The paper was then waxed by passing through a paraffin containing trough so that the finished paper contained 30% by weight of paraffin. The paper thus made was used for the wrapping of pork loins which were placed in the dark at 35° F. for 2 months. Even though the hydroquinone was covered by the paraffin film and not in direct contact with the loins, they were nevertheless substantially stabilized against oxidative deterioration for at the end of the 2 month period, they were in good condition and had a good flavor whereas similar loins wrapped in waxed paper that had not been sized with the hydroquinone before wrapping had a noticeable off-flavor and were considerably darker in color.

The treatment of paper packaging materials with hydroquinone before the waxing thereof is of particular importance because there is avoided any possibility of contact between the packaged organic composition and the hydroquinone due to the paraffin layer. Even though, therefore, the stabilizer used be objectionable if it were to contact the packaged composition such as if hydroquinone or pyrogallol were to be in intimate contact with a packaged food product, and even

though such objectionable stabilizer were not in direct contact with the packaged food product to contaminate it, nevertheless the hydroquinone or pyrogallol under the paraffin film substantially stabilizes that packaged food product.

It is particularly desirable to subject the paper or board following the sizing thereon of the hydroquinone to an elevated temperature of at least 210° F. and preferably to 220° F. or above. Under the conditions of the elevated temperature, the hydroquinone becomes much more effective, which increase in effectiveness is particularly noticeable in the treatment of boards of low quality stock such as of pine board which is so readily susceptible to transferring objectionable cardboard odors to packaged compositions.

#### EXAMPLE VI

A pine stock board was sized with hydroquinone by passing it through a bath containing 10% of hydroquinone by weight. Part of the board thus treated was dried in a vacuum oven at 135° F. and part subjected to a temperature of 220° F. until dried. The boards were then used for the packaging of sweet cookies and held at 98° F. in the dark. It was observed that the cookies packed in the board which was dried at 220° F. kept free of the objectionable "cardboard" odor and flavor for about 40% longer than the cookies packed in the board which was dried at 135° F.

It is not known as to why the heat treatment should so definitely increase the stabilizing value of the aromatic compositions described for it would normally be expected that the heat treatment decrease the effectiveness of the stabilizer. Apparently, however, some reaction occurs whereby the effectiveness of the hydroquinone or similar materials is definitely enhanced by the heat treatment.

It is particularly desirable, therefore, in accordance with this invention for the hydroquinone to be applied at the calender stacks or as a tub sizing and for the paper or board to pass through that bath, and then to subject the paper or board to an elevated temperature of at least 45 212° F. and preferably to 220° F. or higher.

The hydroquinone may much less desirably be added to the beaters but it has been observed that when the addition is made to the beaters, no more than 50% and in most cases much less effectiveness is obtained than where a surface application is made. In the case of the low grade secondary stock boards, and where the stocks in the beaters are subjected to a temperature of about 190° F. and preferably to 210° F. or above, the hydroquinone may be added to the beaters. This is particularly desirable in the treatment of pine stock and other low grade board.

It is undesirable to mix the hydroquinone with the wax and then apply the mixture to the paper or board because of reduction in the moisture-proofness and contamination of the paraffin or wax. Moreover, the results obtained are in most cases not as pronounced as when the hydroquinone is under the paraffin film as described in this invention.

The hydroquinone or similar material used in accordance with this invention does not work on the principle of absorbing light rays responsible for the oxidative deterioration of packaged organic compositions and the paper or board made in accordance with this invention is primarily intended for utilization in the packaging of foodstuffs that are held on grocery store shelves or under refrigeration where they would

not be exposed to such objectionable light rays allegedly responsible for racidity of fats exposed to them.

As stated above, the preferred compounds utilized are absorbed at the surface of the paper sheet material without causing any substantial change in the color or appearance thereof and the stabilizing activity which is obtained appears to arise from catalytic chemical contact action without any light filtration or direct combination with the packaged composition, although there may be a combination with the paper or board or polyhydroxylated aliphatic materials utilized as carriers to give enhanced benefit.

The preferred compounds are those which have a single aromatic ring, preferably a phenyl ring, and which are para substituted.

Where the paper is supercalendered, it is desirable to apply the hydroquinone before the supercalendering operation.

Although it is usually desirable to utilize the hydroquinone or other aromatic compound by itself, as a surfacing, it is also possible to use combinations of the aromatic compounds with lecithin, kephalin, phosphoric acid, phosphatides, glucose, sucrose, lactose or other sugars, and less preferably with the alkali metal phosphates, calcium phosphates, tartaric, citric or other polybasic and/or polyhydroxy aliphatic acid, this combination being utilized particularly in the treatment of secondary stock papers and boards such as pine stock board and where the paper is subjected to an elevated temperature of at least 212° F. and preferably to 220° F. or above after the application of the combination thereto. These added compounds may generally be used in amounts ranging from 5% to 100% of the hydroquinone used.

Upon the accompanying drawing is diagrammatically shown certain aspects of the present invention.

Figure 1 is a diagrammatic transverse sectional view upon an enlarged scale showing a cross section of the paper packaging material after preparation according to the present invention.

Figure 2 shows said packaging material made up into a package and carrying an organic material subject to oxidative deterioration which is only in contact with said paper packaging material over a minor proportion of its own surface and of the surface of the packaging material.

Figure 3 is a diagrammatic layout of the method of applying the antioxidant on the paper and showing also the subsequent heat treatment to which the paper after the application of the antioxidant thereto is subjected.

Referring to Figure 1, A is the surfaced packaging material, a being the surfacing of the antioxidant, such as hydroquinone, applied to the paper base b with or without a subsequent heat treatment to enhance the activity of the antioxidant as a result of the reaction between the antioxidant and the cellulosic packaging material.

In Figure 2, is shown a package made of the surfaced packaging material A containing the crackers which are only in contact with the packaging material A at their edges, leaving a major portion of the area of the crackers exposed to the air inside of the package and to any air which may pass through the walls of the package, where such package is unwaxed or where the wax coating has broken down.

It has been found that, although there is a substantial exposure to air, nevertheless this very slight contact with the activated antioxidant

packaging material has resulted in a communication of the antioxidant activity apparently to the whole body of the organic material, in this case soda crackers, within the package.

In Figure 3, the paper material A is shown as passing through the surfacing bath over the rollers 10, 11 and 12, where the paper picks up the desired amount of the antioxidant in aqueous solution or suspension. After the excess solution has been removed at 12, the paper may be subjected to the heat treatment in the oven E by being passed a large number of times over rollers 13.

It will be noted that the packaged organic products, which in this case are soda crackers or biscuits C, have only their edges C in contact with the coated packaging material A but nevertheless are highly stabilized against oxidative deterioration.

The present application is a continuation in part of applications, Serial No. 144,489, filed May 24, 1937 and Serial No. 190,887, filed February 16, 1938.

Having described my invention, what I claim is:

1. A process of making a flexible sheet wrapping material comprising first applying to the sheet packaging material a surfacing of an antioxidant which is spread over the entire surface thereof and then applying an overcoat of a water repellent coating material, said antioxidant being hydroquinone and said coating material being paraffin.

2. A process of preparing an antioxygenic wrapping paper which comprises passing the paper through a bath containing about 10% hydroquinone and 90% water to obtain complete surface coverage on said paper, drying the paper and then applying an overcoat of a wax covering over the hydroquinone.

3. A flexible sheet wrapping material which has been surfaced with an antioxidant which is spread over the entire surface thereof, and which contains over said surfacing of said antioxidant a water repellent wax material which has been spread over the surface of said packaging material and over the surface of said antioxidant, said antioxidant being hydroquinone and said wax material being paraffin.

4. A process of making a flexible sheet wrapping material which comprises first treating the wrapping material with antioxygenic vanillin and then applying an overcoat of a wax.

5. A process of making a flexible sheet wrapping material which comprises first treating the wrapping material with antioxygenic gallo-tannin and then applying an overcoat of a wax.

6. A flexible sheet wrapping material which has been treated with an antioxygenic compound selected from the group consisting of hydroquinone, guaiacol, pholoroglucinol, resorcinol, pyrogallol, tyrosine, eugenol, thymol, vanillin, gallic acid and gallo-tannin, and which contains an overcoat of a wax.

7. A process of making a flexible sheet wrapping material which comprises first treating the wrapping material with an antioxygenic compound selected from the group consisting of hydroquinone, guaiacol, pholoroglucinol, resorcinol, pyrogallol, tyrosine, eugenol, thymol, vanillin, gallic acid and gallo-tannin, and then applying an overcoat of a wax.

8. A flexible sheet wrapping material which has been treated with an antioxygenic compound selected from the group consisting of hydroquinone, guaiacol, pholoroglucinol, resorcinol, 75

pyrogallol, tyrosine, eugenol, thymol, vanillin, gallic acid and gallo-tannin, and which contains an overcoat of a paraffin.

9. A process of making a flexible sheet wrapping material which comprises first treating the wrapping material with an antioxygenic com-

pound selected from the group consisting of hydroquinone, guaiacol, phloroglucinol, resorcinol, pyrogallol, tyrosine, eugenol, thymol, vanillin, gallic acid and gallo-tannin, and then applying an overcoat of a paraffin. 5

SIDNEY MUSHER.